

Patented June 9, 1925.

1,540,867

# UNITED STATES PATENT OFFICE.

GUSTAV SCHREIBER, OF GRIESHEIM-ON-THE-MAIN, AND ADOLF BECK, OF SCHWANHEIM-ON-THE-MAIN, GERMANY, ASSIGNEES TO CHEMISCHE FABRIK GRIESHEIM ELEKTRON, OF FRANKFORT-ON-THE-MAIN, GERMANY.

## METHOD OF TREATING MOLTEN MAGNESIUM.

No Drawing.

Application filed October 29, 1923. Serial No. 671,403.

*To all whom it may concern:*

Be it known that we, GUSTAV SCHREIBER and ADOLF BECK, citizens of Germany, residing at Griesheim-on-the-Main and Schwandheim-on-the-Main, Germany, respectively, have invented certain new and useful Improvements in Methods of Treating Molten Magnesium, of which the following is a specification.

10 The invention refers to a method of treating molten magnesium and its alloys with a view to protecting them against oxidation.

In treating and handling magnesium and 15 alloys rich in magnesium in molten condition, it is important that the metal or alloy treated be protected against oxidation. This is not only a question of protecting them against an oxidation resulting in a burning 20 of the metal with an open flame, but also against slow oxidations causing films of an oxid to be formed on the metal. All such films impair the quality of the metal as they interrupt the homogeneity of the metal and 25 reduce its mechanical strength in the finished articles.

We have ascertained that it is possible to 30 absolutely prevent oxidation of magnesium and its alloys by placing sulphur on the bright surface of the metal, provided that this be done at temperatures which are near or above the melting point, but not so high as to cause the metal to react with the sulphur. We have observed that this range 35 of temperatures is wide enough to permit the slight overheating of the metal beyond the melting point which is required as a rule in all casting operations.

The effective principle underlying our invention 40 consists in causing an atmosphere of sulphur vapour to be formed above the metal, another atmosphere of SO<sub>2</sub> being formed above the first atmosphere by combustion.

45 The sulphur can be placed on the surface of the metal in different manner, either in solid or in molten condition or as vapour. We have found it to be preferable to dust or spray the sulphur onto the metal, for instance by dusting fine sulphur powder 50 through a linen bag by shaking. We may, however, also direct a spray comprising sulphur powder against the metal. The dusting or spraying can be effected while the

metal is at rest or in motion, for instance 55 during the melting down in crucibles or pans or the like, or during casting, the jet of sulphur powder being then directed onto the crucibles, the flowing metal and the molds.

We have further utilized our novel method as a means for extinguishing the flame of burning magnesium or magnesium alloys. It is true that the parts of the metal which are already burning will react with the sulphur, magnesium sulfide being formed, but that portion of the metal which is merely heated and in the course of melting down, is protected by the sulphur against catching fire, so that fires arising in crucibles or in 60 the heaps of metal chips which have caught fire can easily and safely be extinguished. In the latter case, it is not always necessary to employ only sulphur; we have found that in such a case the sulphur can be diluted 65 by additions of inert materials, such as magnesia or sand which need not be perfectly dry.

We wish it to be understood that we do not desire to be limited to the exact means 70 or sequences of steps described, for obvious modifications will occur to a person skilled in the art.

We claim:

1. The method of protecting molten magnesium and its alloys against burning, comprising placing sulphur onto the surface of the molten metal.

2. The method of protecting molten magnesium and its alloys against burning comprising placing sulphur powder onto the surface of the molten metal.

3. The method of protecting molten magnesium and its alloys against burning comprising spraying sulphur powder onto the 95 surface of the molten metal.

4. The method of protecting molten magnesium and its alloys against burning comprising spraying a mixture of sulphur powder and an inert material onto the 100 surface of the molten metal.

In testimony whereof we affix our signatures.

GUSTAV SCHREIBER.  
ADOLF BECK.

Witnesses:

IVAN LAVRETOKY,  
H. SCHICHERT.